# EUROPEAN PATENT SPECIFICATION

(11) **EP 3 809 600 B1**
(45) Date of publication and mention of the grant of the patent: **08.03.2023**
(21) Application number: 19823534.3
(22) Date of filing: 23.04.2019
(51) Int. Cl.: H04B 3/14

(54) **HEATABLE PANEL AND ITS MANUFACTURING METHOD**
BEHEIZBARE PLATTE UND IHR HERSTELLUNGSVERFAHREN
PANNEAU CHAUFFABLE ET PROCÉDÉ DE FABRICATION DE CELUI-CI

(30) Priority: 18.06.2018 ES 201830593
(43) Date of publication of application: 21.04.2021
(73) Proprietor: AIMPLAS - Asociación de Investigación de Materiales Plásticos y Conexas, 46980 Paterna-Valencia (ES)
(72) Inventor: GALINDO GALIANA, Begoña, 46980 Paterna (Valencia) (ES); GUTIÉRREZ ARAGONÉS, Vanessa, 46980 Paterna (Valencia) (ES); MARTÍNEZ SANZ, Vicent, 46980 Paterna (Valencia) (ES)
(74) Representative: Ungria López, Javier
(86) International application number: PCT/ES2019/070276
(87) International publication number: WO 2019/243644

(56) References cited:
- EP-A1- 3 288 890
- EP-A2- 0 437 239
- WO-A1-2009/040774
- CN-A- 104 788 818
- US-A1- 2010 213 189
- US-A1- 2017 006 664
- P. NOORUNNISA KHANAM et al.: "Electrical properties of graphene polymer nanocomposites." In: "GRAPHENE-BASED POLYMER NANOCOMPOSITES IN ELECTRONICS", 20 January 2015 (2015-01-20), Springer link, XP055664565, ISBN: 978-3-319-13875-6 pages 25-47, DOI: 10.1007/978-3-319-13875-6_2,
- GARY THOMAS: "Recycling of polypropylene", azocleantech.com, 19 October 2012 (2012-10-19), XP009520857, Retrieved from the Internet: URL:http://web.archive.org/web/20121019101 645/https://www.azocleantech.com/article.a spx?ArticleID=240 [retrieved on 2019-05-27]

## Description

### Object of the invention and field of application

The present invention relates to heatable panels produced by means of conventional plastic transformation processes based on conductive thermoplastic compounds. The panel is heated as a result of Joule effect whereby an electrically conductive material is heated when an electric current is applied. These panels can be used as a heating system in different sectors such as automotive, construction, aerospace, and packaging sectors. The panels can be obtained by means of extrusion, injection, or compression molding and then shaped to enable adapting to different geometries.

### Background of the invention

Different protected systems to be used as Joule heating or resistive heating are known up until now. None of the reviewed inventions refer to thermoplastic polymers obtained by means of extrusion, injection, or compression, since the high electrical conductivity required to achieve the Joule effect is much more difficult to obtain by means of conventional plastic processing processes. Several inventions, the novelty of which lies in the development of conductive coatings on different substrates, have thus been found.

Invention ES2574622 uses, as a heatable material, a thermosetting elastomer with a high percentage of carbon nanotubes (CNTs) (between 20 and 45% by weight) added as additive. This elastomer is used as a coating in different substrates. The invention indicates the importance of copper electrodes which are deposited by means of electrochemical electrodeposition on the conductive material.

In invention WO 2007089118, a highly conductive film that can be heated is obtained by spraying an aqueous solution of carbon nanotubes (CNTs) on a polymer sheet. Invention DE102011086448(A1) is also based on the deposition of layers of an aqueous solution of carbon nanotubes (CNTs) for obtaining a heatable coating.

Invention WO2002076805 A1 describes a steering wheel that can be heated by means of applying carbon particle-based conductive coatings. In invention ES2402034B1, work is also performed with different layers of conductive coatings, and it also contemplates the encapsulation of heatable elements and electrodes.

Inventions US2005172950 and WO 2009011674 relate to heatable fabrics or clothing. The former is based on impregnating fabrics with conductive coatings and the latter obtains the conductive fabric from long carbon nanotube fibers.

In invention DE102007004953 (A1), carbon nanotubes and intrinsically conductive polymers are used as a heatable coating in glasses.

In invention ES 2537400 B1, conductive coatings are applied in heatable automobile elements, specifically in rear-view mirrors.

Claim 2 of patent DE102011003012 refers to a cross-linked polymer and the example specifies the use of a silicone. These materials are thermally stable and cannot be processed by extrusion. Thermoplastic polymers can be partially cross-linked to obtain an extruded sheet but, in that case, they cannot be melted again, leading to the inability to recycle same.

The patent application EP 0437239 A2 is also considered prior art and it discloses a heated panel or sheet, capable of producing heat energy when an electric current is applied. Furthermore, this document describes the method for obtaining such panel that comprises a first step of mixing crystalline resin with the electrically conductive particles, and a second step, wherein the mixture obtained in the first step is kneaded, cross linked and molded to produce the desire form under the action of organic peroxide.

In the present invention the materials are in no case cross-linked, with recyclability being a very novel feature of the panel. Furthermore, it relates to soft materials such as silicone, whereas the materials of the present invention are rigid panels.

The materials developed in the present invention have a much lower resistivity, being much more conductive than the materials specified in said German invention DE102011003012. The low conductivity conditions the design of the electrodes, resulting in said electrodes having to be relatively close and have a large size (similar to the geometry of the heatable sheet).

In invention GR1449261, the process of obtaining a highly conductive film is very different from that developed in the present invention. It is based on annealing which is performed on the polymer after the extrusion of the film. This annealing can last up to 24 h.

The present invention does not contemplate this technology because good conductivity is achieved by properly dispersing the conductive charge and correctly processing the material to obtain the final film or part with the desired conductive properties. Therefore, a PTC plastic is obtained by means of conventional processes as a result of the good dispersion of the conductive particles which are achieved by applying certain specific processing conditions, which also allows producing larger geometries with a greater distance of the electrodes.

Invention CN201610317174 relates to solvent-based conductive pastes without being thermoplastic polymers. The polymeric material produced by means of extrusion is the (non-conductive) substrate on which the conductive paste is applied. It is a functional ink printing process that is very different from thermoplastic processing.

Therefore, the inventions that are found are based on the application of conductive paints or varnishes that finally form a conductive coating or on the extrusion of materials with worse electrical conductivities, which subsequently makes the configuration of the electrodes difficult and complicated. The application of coatings is a manual process and the final behavior of the heating element depends on different factors, such as: the number of layers of the conductive solution or paint, the worker who applies the paint, the homogeneity of the solution, given that if the conductive particles decant over time, the first applied layer may have a much higher concentration of conductive particles than the last applied layer. Therefore, the heating homogeneity and the reproducibility of the heating elements produced are not stable.

In the present invention, the conductive particles are dispersed in the thermoplastic die in a co-rotating twin-screw extruder. A homogeneous nanocompound with high electrical conductivity is obtained, allowing the electrodes to be positioned at a great distance. In a subsequent processing, this material is melted to obtain a conductive sheet. Said process can be an extrusion, compression, or injection. The obtained part will have a homogeneous concentration of conductive particles, ensuring a reproducible and homogeneous behavior. Furthermore, as it is based on thermoplastic materials, the sheet can be ground and reprocessed, assuring recycling at the end of the product's service life. Recycling is not contemplated in the state of the art since different materials and thermosetting coatings that do not allow recycling are combined.

Unlike the inventions mentioned in the prior art, the materials developed and the manufacturing process carried out in the present invention provide a lower resistivity of the conductive sheet of 10¹ Ohm.cm, which is much lower with respect to patent DE102011003012A1, which mentions resistances between 10³ and 10⁶ ohm.cm, implying a greater conduction by the developed panel.

### Description of the invention

The present invention has been devised as a heating panel which uses, as a power source, electrical energy that is to be converted into thermal energy. The novelty lies in the type of material making up the heatable panel and in its manufacturing process.

The conceived solution is based on obtaining a sheet of recyclable, lightweight conductive polymer to be used in a wide variety of designs depending on the sizes and geometries required according to the application.

The polymer materials are usually insulating materials; however, as a result of the addition of conductive additives, they can change their thermal and electrical properties and replace heat-generating metallic resistors when this type of heating is required.

The heatable panel, according claim 1, produces thermal energy when an electric current is applied, such that in order to carry out this process, the panel comprises:
- a sheet made of thermoplastic material with temperature conducting particles added as additive, providing the sheet with a PTC (Positive Temperature Coefficient) behavior, wherein the geometry of the sheet can be adaptable by means of thermoforming processes used in the manufacture thereof and wherein said sheet is recyclable;
- metallic electrodes mechanically connected to the sheet and configured for applying an electric current going through said sheet;
- a first temperature- and electricity-insulating layer configured for preventing heat energy losses in the direction opposite the desired direction;
- a second electricity-insulating layer configured for preventing direct contact with the sheet; and
- a thermocouple sensor attached to the sheet configured for measuring the internal temperature of the heatable panel;
such that the sheet is attached to the first insulating layer on one side and to the second insulating layer on the opposite side. The metallic electrodes are attached on opposite longitudinal ends of the sheet and the thermocouple sensor is attached in the central part of the sheet.

All these components forming the heatable panel, i.e., the sheet, the first insulating layer, the second insulating layer, the thermocouple sensor, and the metallic electrodes, are reusable to form part of another heatable panel or to form part of another system.

Since the sheet has a PTC thermistor behavior, when an electrical current is applied to the metallic electrodes, the sheet works by increasing the electrical resistance with the increase of temperature. In other words, once the desired temperature is reached, it stabilizes and no temperature peaks are generated, making it a safe heating system. This feature gives it the particularity of being self-regulating, dispensing with the need for thermostats that are necessary in other heating systems.

The conductive particles added as additive to the thermoplastic material of the sheet have directly proportional percentages in the mixture with the thermoplastic material, depending on the final temperature required by the heatable panel and on the type of conductive particles used. Once the material has been formulated, the temperature of the panels can be regulated by adapting the input voltage or cutting off the current supply, without having to adapt the formulation to each of the applications.

These temperature conducting particles of the sheet can be carbon black, graphite, graphene, carbon nanotubes, or a combination of the foregoing.

In one embodiment, the conductive particles added as additive to the thermoplastic material of the sheet are carbon nanotubes and have a concentration comprised between 5 and 10% with respect to the total weight of the sheet.

In other embodiments, when the conductive particles are of graphite material, the concentration is comprised between 20 and 40%, when they are of carbon black, the concentration is between 10 and 30%, when they are of graphene, between 3 and 10%, all these percentages being with respect to the total weight of the mixture forming the sheet.

The thermoplastic materials of the sheet can be polyolefins, polyesters, polyamides, thermoplastic elastomers, polysulfones, polyetherimides, or a combination of all the foregoing, since all of them allow mixing with the temperature conducting particles and have structural and mechanical characteristics suitable for the use of the heatable panel, although a type of polyolefin, i.e., polypropylene, is preferably used.

Furthermore, since it is a polymeric compound, the composite layer can adopt several forms by means of thermoforming, obtaining a lightweight final compound, allowing the use thereof for spaces with special geometries. Furthermore, machining operations can be applied thereto to make the adjustment with other elements.

In one embodiment, the heatable panel also comprises a coating fabric partially or completely covering the panel, said coating fabric being an electrically insulating material that is resistant to temperature changes and selected depending on the characteristics of the installation of the panel.

The conductive materials of the metallic electrodes can be copper or silver, although other metallic materials that can be mechanically attached to the sheet to be reused can be selected.

The manufacturing process for manufacturing the sheet made of thermoplastic material with temperature conducting particles added as additive is carried out by means of plastic and thermoplastic transformation processes.

To that end, the conductive particles in the form of powder and the thermoplastic material in the form of pellets are first introduced in a heated container of a co-rotating twin-screw extruder.

Once the conductive particles and the thermoplastic material have been introduced in the container, they are hot mixed, melting the thermoplastic material in the extruder, to achieve a homogeneous mixture, applying a specific mechanical energy of at least 0.5 kWh/kg while melting the thermoplastic material.

The purpose of this process is to disperse the conductive charge in the polymer die to achieve optimal electrical properties homogeneously throughout the volume of the sheet.

To achieve optimum dispersion, the thermoplastic material is melted at a temperature of 210°C, for the preferred case of a polypropylene die, and the screws rotate at a speed greater than 600 rpm, for a material input of 10 kilograms per hour in the co-rotating extruder measuring 25 mm diameter and with a length to diameter ratio equal to 40.

Once a homogeneous mixture is achieved, said mixture of molten plastic with the conductive particles is passed through an extruder head configured for generating filaments of thermoplastic material with conductive particles added as additive.

Once cooled, these filaments of thermoplastic material with added additive are cut using a shear to obtain pellets of said material.

In order not to lose electrical conductivity, processing must be optimized, assuring slow cooling of the material at the head outlet. The calender rollers must be at a high temperature, assuring that the carbon nanotubes have enough time to be distributed into the polymer die and form the conductive network.

In a subsequent manufacturing process, said pellets are melted to obtain the sheet of heatable panel by means of a new extrusion, drawing, roller lamination, or a combination of these manufacturing processes, all these processes being hot processes to facilitate the molding of the sheet, although it can also be performed by means of injection into plastic dies or compression molding. With these manufacturing processes, the geometry of the sheet can be adaptable to any geometry depending on the shape and size requirements.

In another embodiment, the thermoplastic material conductive sheet with conductive particles added as additive can be obtained in a single step, coupling a co-rotating extruder to a flat sheet head. The panel is therefore more cost-effective and faster to manufacture.

Furthermore, as it is based on thermoplastic materials, the sheet can be ground to obtain pellets again, and reprocessed, assuring recycling at the end of the product's service life. This recycling is not contemplated in the prior art found since different embedded materials and thermosetting coatings that do not allow recycling are combined.

In this described sheet manufacturing method, the conductive particles do not coat any material, but are dispersed in the die of the co-rotating twin-screw extruder with the thermoplastic material, unlike these inventions mentioned in the prior art, so the materials developed in the present invention obtain the mentioned resistivity of 10¹ Ohm.cm, and a greater thermal conduction.

This good conductivity is only achieved by properly dispersing the conductive charge and correctly processing the conductive particles to obtain the sheet with the desired conductive properties.

Therefore, with this process a PTC plastic sheet is achieved by means of manufacturing processes as a result of the dispersion of the conductive particles, which are achieved by applying certain specific processing conditions. This also allows producing geometries having a larger size than those found and a greater distance between the electrodes.

When all the materials have been manufactured, the heating panel is constructed by means of custom machining according to the desired geometry of the final panel or by means of thermoforming, connecting the electrodes to the sheet and placing the insulation layers on the sides of said sheet.

Once these layers have been attached to the sheet, the assembly is covered by means of the coating fabric customized according to the design and the final application, with fabrics that are resistant to temperature changes or possible iterations that they may have with the exterior to provide a finish suitable for use.

All the parts of the heating panel are therefore completely recyclable due to their nature and reusable for the same or another application.

### BRIEF DESCRIPTION OF THE FIGURES

- Figure 1 shows an elevation view and another profile view of the heatable panel.
- Figure 2 shows the temperature reached by heatable panels with heat conducting sheets of different sizes and geometries.
- Figure 3 shows a graph indicating how the temperature levels of the material of a sheet manufactured from polypropylene with carbon nanotubes vary when 48 V are applied starting from a temperature of - 21°C.

### PREFERRED DESCRIPTION OF THE INVENTION

As can be seen in Figure 1, the heatable panel of the present invention is formed by a sheet (1), manufactured from a thermoplastic material, metallic electrodes (6) mechanically connected on the sides to the sheet (1), a first insulating layer (3) located on one side of the sheet (1), preventing the sheet from losing temperature on the side opposite the desired side and also preventing the passage of electric current on that side, a second electricity-insulating layer (2) for limiting the passage of electric current on the opposite side of the sheet (1) where heat is emitted, and a thermocouple sensor (5) attached to the sheet (1) measuring the internal temperature of the heatable panel.

In the preferred embodiment, said heatable panel is partially or completely coated by a coating fabric (4) made of an electrically insulating material for two purposes. Preventing a user who is close to the panel from coming into unwanted contact with the electrically conductive heatable sheet (1) and providing a finish according to the panel installation location.

This coating fabric (4) can be of many types, but a natural fabric is preferably selected.

Despite being made from a thermoplastic material, the sheet (1) is capable of emitting heat because electrically conductive particles are added as additive, providing the sheet (1) with PTC behavior. These temperature conducting particles of the sheet (1) can be of different types such as carbon black, graphite, graphene, carbon nanotubes, and a combination of the foregoing, carbon nanotubes (CNTs) preferably being used due to their heat conduction properties.

The percentage of these carbon nanotube particles is comprised between 5 and 10% with respect to the total weight of the sheet, which is completed with thermoplastic materials selected from polyolefins, polyesters, polyamides, thermoplastic elastomers, polysulfone, polyetherimide, or a combination of all of the foregoing, although polypropylene, a compound from the groups of polyolefins, is preferably used.

Figure 2 shows the temperature that the heatable panel can reach using carbon nanotubes (CNTs) in different percentages and different sizes as additive particle, so that the higher the percentage of nanotubes, the higher the temperature reached by the panel.

The thermoplastic material used in this case, shown in Figure 2, is a polypropylene in which different percentages of carbon nanotubes (CNTs) from 3% to 10% by weight have been mixed. Different temperatures in degree Celsius are generated by applying a voltage of 48 V to the heatable panel, reaching up to 100°C if the panel has a smaller surface with sides measuring 15 x 15 cm.

In the graph of Figure 3, the operation of a sheet manufactured from polypropylene with carbon nanotubes is shown, to which a voltage of 48 volts has been applied gradually during the first minute, establishing that constant voltage until minute 6. Due to the applied load, the temperature of the panel begins to go up in a logarithmic growth, going from -21°C to 75°C within those 6 minutes, in which the indicated voltage is applied. The temperature drops gradually in an exponential decrease when the voltage is removed.

With these materials used in the sheet of the heatable panel, the test of which is shown in Figure 3, 45°C is reached within 4 minutes starting at a temperature of -21°C.

The energy consumption of said heatable panel is 120 W for a rectangular geometry measuring 350 cm on one side by 250 cm on the other side and by 2 cm wide, applying 48 V and 64 W, for the same geometry, applying 24 V. For a smaller geometry of a square panel measuring 15 cm on each side and by 1 cm wide, the energy consumption is 20 W at 48 V and 5 W at 24 V.

To manufacture the sheet (1) a series of processes is followed to achieve the mentioned operating characteristics. Since the sheet (1) is formed by a thermoplastic material and particles added as additive, firstly the mixing of both components is performed, so that they are blended together in the state of pellets and powder, and heated to melt the plastic material, where it is stirred inside an extruder applying a specific mechanical energy of at least 0.5 kWh/kg.

The thermoplastic material is melted at a temperature of at least 210°C when polypropylene is used and the screws rotate at a speed of at least 600 rpm for a material input of 10 kilograms per hour in a co-rotating extruder measuring 25 mm in diameter and with a length to diameter ratio equal to 40.

Once the correct homogenization of the mixture has been achieved, the material is extruded to obtain filaments that are cooled and solidified in rollers, to be subsequently cut using a shear and to obtain new pellets but from the mixture of components.

Said pellets are used to obtain the sheet (1) following one or different plastic transformation processes, such as extrusion, drawing, compression molding, roller lamination, or die injection.

Once the sheet (1) has been manufactured, it is attached to the rest of the components forming the heatable panel and is ready for use.

### EXAMPLES

### Example 1: Polypropylene- and carbon nanotube (CNT)-based heatable panel

The present example refers to a sheet made of polypropylene and carbon nanotubes obtained by means of flat sheet extrusion. In this process, the plastic material is melted by means of heat and shear in an extruder and is forced to pass through a head, giving it the shape of a sheet. The sheet is passed through a roller system or calender. The cooling of the material is controlled by varying the temperature of these rollers.

The key parameters for processing the sheet with high electrical conductivity by means of extrusion are shown in Table 1.

**Table 1: Optional extrusion parameters**

| **Parameter** | **Value** |
|---|---|
| Area 1 (°C) | 180 |
| Area 2 (°C) | 185 |
| Area 3 (°C) | 195 |
| Area 4 (°C) | 200 |
| Area 5 (°C) | 210 |
| Head (°C) | 220 |
| Melt temperature (°C) | 211 |
| Pressure (bar) | 57 |
| Speed (rpm) | 60 |
| Torque (N/m2) | 4.5 - 23% |
| Drawing (%) | 1.0 |
| *Die Gap (µm)* (Nozzle opening) | 900 |
| Roller temperature (°C) | 80 |
| Film thickness (µm) | 900 |

The percentage of carbon nanotubes is determined according to the temperature of use required by the application. The optimal range being between 5 and 10% of nanotubes to reach temperatures between 25 and 100°C.

### Example 2: Polypropylene- and graphite-based heatable panel

In this second example, the sheet is obtained by means of compression molding. The main parameters involved in the process are the pressure exerted on the mold, the cycle time, and the temperature during processing.

Table 2 shows the processing conditions to achieve optimum electrical conductivity in the graphite plates.

**Table 2: Compression molding processing parameters**

| Units | **BIPOLAR** | | | | |
|---|---|---|---|---|---|
| Min | E1 | E2 | E3 | E4 | E5 |
| | 4 | 2 | 2 | 4 | 15 |
| bar | P1 | P2 | P3 | P4 | P5 |
| | 4 | 40 | 75 | 150 | 70 |
| °C | T1 | T2 | Dry samples for 2 h at 80°C | | |
| | 190 | 190 | | | |

Table 3 shows the temperatures reached in three areas of the heatable panel when a certain voltage is applied. In this case, the panels have a geometry of 15 x 15 cm and they were obtained by means of compression molding.

**Table 3: Thermal behavior of panels containing polypropylene and graphite**

| | **PP+20%graphite** | **PP+30%graphite** | **PP+40%graphite** |
|---|---|---|---|
| T1 | 45.9 | 96.6 | 102 |
| T2 | 45.7 | 100 | 86.9 |
| T3 | 46.3 | 80.6 | 60.7 |
| V | 48 | 48 | 38 |
| Current (A) | 0.24 | 5.12 | 5.11 |
| Power (W) | 11.52 | 245 | 195 |

## Claims

1. A heatable panel adapted to produce heat energy when an electric current is applied and it comprises:
- metallic electrodes (6) mechanically connected to a sheet (1) and configured for applying an electric current going through said sheet (1);
- the metallic electrodes (6) are on opposite longitudinal ends of said sheet (1);
is **characterized in that** it comprises:
- the sheet (1) made of thermoplastic material which is selected from the group consisting of polyolefins, polyesters, polyamides, thermoplastic elastomers, polysulfone, polyetherimide, and a combination of all the foregoing, with electrically conductive particles added as additive, providing the sheet (1) with a PTC behavior;
- a first temperature- and electricity-insulating layer (3) configured for preventing heat energy losses in the direction opposite the desired direction;
- a second electricity-insulating layer (2) configured for preventing direct contact with the sheet (1); and
- a thermocouple sensor (5) attached to the sheet (1) configured for measuring the internal temperature of the heatable panel;
wherein the sheet (1) is attached to:
- the first insulating layer (3) on one side of said sheet (1);
- the second insulating layer (2) on the opposite side of the attachment of said sheet (1) with the first insulating layer (3);
and
- the thermocouple sensor (5) in the central part of the sheet (1).

2. The heatable panel according to claim 1, **characterized in that** the temperature conducting particles of the sheet (1) are selected from the group consisting of carbon black, graphite, graphene, carbon nanotubes and a combination of the foregoing.

3. The heatable panel according to claim 2, **characterized in that** the conductive particles added as additive to the thermoplastic material of the sheet (1) are carbon nanotubes with a concentration comprised between 5 and 10% with respect to the total weight of the sheet.

4. The heatable panel according to claim 2, **characterized in that** the conductive particles added as additive to the thermoplastic material of the sheet (1) are of graphite material with a concentration comprised between 20 and 40% with respect to the total weight of the sheet.

5. The heatable panel according to claim 2, **characterized in that** the conductive particles added as additive to the thermoplastic material of the sheet (1) are of carbon black with a concentration comprised between 10 and 30% with respect to the total weight of the sheet.

6. The heatable panel according to claim 2, **characterized in that** the conductive particles added as additive to the thermoplastic material of the sheet (1) are of graphene with a concentration comprised between 3 and 10% with respect to the total weight of the sheet.

7. The heatable panel according to any one of the preceding claims, **characterized in that** the heatable panel additionally comprises a coating fabric (4) partially or completely covering the panel, said coating fabric (4) being an electrically insulating material selected from a group consisting of polyvinyl chloride, polyurethane, natural fabrics, and a combination of all the foregoing.

8. The heatable panel according to any one of the preceding claims, **characterized in that** the conductive materials of the metallic electrodes (6) are selected from the group consisting of copper and silver.

## Patentansprüche

1. Beheizbare Platte, die so eingerichtet ist, dass sie Wärmeenergie erzeugt, wenn ein elektrischer Strom angelegt wird, und sie umfasst:
- Elektroden (6) aus Metall, die mechanisch mit einer Folie (1) verbunden und zum Anlegen eines durch die Folie (1) fließenden elektrischen Stroms ausgeführt sind,
- wobei sich die Elektroden (6) aus Metall an gegenüberliegenden Längsenden der Folie (1) befinden;
**dadurch gekennzeichnet, dass** sie umfasst:
- die Folie (1), die aus einem thermoplastischen Material besteht, das aus der Gruppe ausgewählt wird, die aus Polyolefinen, Polyestern, Polyamiden, thermoplastischen Elastomeren, Polysulfon, Polyetherimid sowie einer Kombination aus allen aufgeführten Materialien besteht, wobei elektrisch leitende Teilchen als Zusatzstoff zugesetzt sind, der der Folie (1) ein PTC-Verhalten verleiht;
- eine erste thermisch und elektrisch isolierende Schicht (3), die so ausgeführt ist, dass sie Verluste von Wärmeenergie in der Richtung entgegengesetzt zu der gewünschten Richtung verhindert;
- eine zweite elektrisch isolierende Schicht (2), die so ausgeführt ist, dass sie direkten Kontakt mit der Folie (1) verhindert; sowie
- einen Thermoelement-Sensor (5), der an der Folie (1) angebracht und zum Messen der Innentemperatur der beheizbaren Platte ausgeführt ist;
wobei die Folie (1) angebracht ist an:
- der ersten isolierenden Schicht (3) an einer Seite der Folie (1);
- der zweiten isolierenden Schicht (2) an der der Anbringung der Folie (1) an der ersten isolierenden Schicht (3) gegenüberliegenden Seite;
und
- dem Thermoelement-Sensor (5) in dem mittleren Teil der Folie (1).

2. Beheizbare Platte nach Anspruch 1, **dadurch gekennzeichnet, dass** die wärmeleitenden Teilchen der Folie (1) aus der Gruppe ausgewählt werden, die aus Ruß, Graphit, Graphen, Kohlenstoff-Nanoröhren und einer Kombination daraus besteht.

3. Beheizbare Platte nach Anspruch 2, **dadurch gekennzeichnet, dass** die leitfähigen Teilchen, die dem thermoplastischen Material der Folie (1) als Zusatzstoff zugesetzt werden, Kohlenstoff-Nanoröhren mit einer Konzentration zwischen 5 und 10 %, bezogen auf das Gesamtgewicht der Folie, sind.

4. Beheizbare Platte nach Anspruch 2, **dadurch gekennzeichnet, dass** die leitfähigen Teilchen, die dem thermoplastischen Material der Folie (1) als Zusatzstoff zugesetzt werden, aus Graphitmaterial mit einer Konzentration zwischen 20 und 40 %, bezogen auf das Gesamtgewicht der Folie, bestehen.

5. Beheizbare Platte nach Anspruch 2, **dadurch gekennzeichnet, dass** die leitfähigen Teilchen, die dem thermoplastischen Material der Folie (1) als Zusatzstoff zugesetzt werden, aus Ruß mit einer Konzentration zwischen 10 und 30 %, bezogen auf das Gesamtgewicht der Folie, bestehen.

6. Beheizbare Platte nach Anspruch 2, **dadurch gekennzeichnet, dass** die leitfähigen Teilchen, die dem thermoplastischen Material der Folie (1) als Zusatzstoff zugesetzt werden, aus Graphen mit einer Konzentration zwischen 3 und 10 %, bezogen auf das Gesamtgewicht der Folie, bestehen.

7. Beheizbare Platte nach einem der vorangehenden Ansprüche, **dadurch gekennzeichnet, dass** die beheizbare Platte zusätzlich ein Beschichtungsgewebe (4) umfasst, das die Platte teilweise oder vollständig bedeckt, wobei das Beschichtungsgewebe (4) ein elektrisch isolierendes Material ist, das aus einer Gruppe ausgewählt wird, die aus Polyvinylchlorid, Polyurethan, natürlichen Geweben sowie einer Kombination aus allen aufgeführten Materialien besteht.

8. Beheizbare Platte nach einem der vorangehenden Ansprüche, **dadurch gekennzeichnet, dass** die leitenden Materialien der Elektroden (6) aus Metall aus der Gruppe ausgewählt werden, die aus Kupfer und Silber besteht.

## Revendications

1. Panneau chauffable adapté pour produire de l'énergie thermique lorsqu'un courant électrique est appliqué et qui comprend :
- des électrodes métalliques (6) mécaniquement raccordées à une feuille (1) et configurées pour appliquer un courant électrique passant à travers ladite feuille (1) ;
- les électrodes métalliques (6) se trouvent sur des extrémités longitudinales opposées de ladite feuille (1) ;
est **caractérisé en ce qu'**il comprend :
- la feuille (1) constituée de matériau thermoplastique qui est choisie dans le groupe consistant en polyoléfines, polyesters, polyamides, élastomères thermoplastiques, polysulfone, polyétherimide, et une combinaison de tous les précédents, avec des particules électriquement conductrices ajoutées comme additif, munissant la feuille (1) d'un comportement PTC ;
- une première couche isolante à la température et l'électricité (3) configurée pour éviter des pertes d'énergie thermique dans la direction opposée à la direction souhaitée ;
- une seconde couche isolante à l'électricité (2) configurée pour éviter un contact direct avec la feuille (1) ; et
- un capteur de thermocouple (5) fixé à la feuille (1) configuré pour mesurer la température interne du panneau chauffable ;
dans lequel la feuille (1) est fixée à :
- la première couche isolante (3) sur un côté de ladite feuille (1) ;
- la seconde couche isolante (2) sur le côté opposé de la fixation de ladite feuille (1) avec la première couche isolante (3) ;
et
- le capteur de thermocouple (5) dans la partie centrale de la feuille (1).

2. Panneau chauffable selon la revendication 1, **caractérisé en ce que** les particules conductrices de température de la feuille (1) sont choisies dans le groupe consistant en noir de carbone, graphite, graphène, nanotubes de carbone et une combinaison des précédents.

3. Panneau chauffable selon la revendication 2, **caractérisé en ce que** les particules conductrices ajoutées comme additif au matériau thermoplastique de la feuille (1) sont des nanotubes de carbone avec une concentration comprise entre 5 et 10 % par rapport à la masse totale de la feuille.

4. Panneau chauffable selon la revendication 2, **caractérisé en ce que** les particules conductrices ajoutées comme additif au matériau thermoplastique de la feuille (1) sont constituées de matériau de graphite avec une concentration comprise entre 20 et 40 % par rapport à la masse totale de la feuille.

5. Panneau chauffable selon la revendication 2, **caractérisé en ce que** les particules conductrices ajoutées comme additif au matériau thermoplastique de la feuille (1) sont constituées de noir de carbone avec une concentration comprise entre 10 et 30 % par rapport à la masse totale de la feuille.

6. Panneau chauffable selon la revendication 2, **caractérisé en ce que** les particules conductrices ajoutées comme additif au matériau thermoplastique de la feuille (1) sont constituées de graphène avec une concentration comprise entre 3 et 10 % par rapport à la masse totale de la feuille.

7. Panneau chauffable selon l'une quelconque des revendications précédentes, **caractérisé en ce que** le panneau chauffable comprend de plus un textile de revêtement (4) recouvrant partiellement ou complètement le panneau, ledit textile de revêtement (4) étant un matériau électriquement isolant choisi dans un groupe consistant en poly(chlorure de vinyle), polyuréthane, textiles naturels, et une combinaison de tous les précédents.

8. Panneau chauffable selon l'une quelconque des revendications précédentes, **caractérisé en ce que** les matériaux conducteurs des électrodes métalliques (6) sont choisis dans le groupe consistant en cuivre et argent.
